

Aug. 9, 1932.

R. THURM

1,871,245

PROCESS OF MAKING VISCOSE

Filed Oct. 26, 1931



Richard Thurm  
INVENTOR

## UNITED STATES PATENT OFFICE

RICHARD THURM, OF SAGINAW, MICHIGAN, ASSIGNOR TO BAKER PERKINS COMPANY, INC., OF SAGINAW, MICHIGAN, A CORPORATION OF NEW YORK

## PROCESS OF MAKING VISCOSE

Application filed October 26, 1931. Serial No. 571,134.

This invention relates to a process of manufacturing viscose such as is used in the manufacture of rayon, cellophane, etc., and pertains more particularly to those steps in the process which come between the soaking of the cellulose sheet from which the viscose is made and the process of spinning into rayon threads or castings into cellophane sheets.

The prime object of this invention is to provide a process wherein several of the steps used heretofore are eliminated, thus saving considerable time in the manufacture, saving equipment, and power used to operate this equipment, eliminating much of the handling, and also making larger batches than has heretofore been possible.

A further object of the invention is to provide a viscose which is easily filterable and which will produce a stronger, more uniform rayon thread, and a clearer more perfect sheet of cellophane.

A still further object is to provide a process in which much of the danger of heating and spoiling the viscose is eliminated and in which every batch will be uniform.

With these and certain other objects, which will appear later in the specification, my invention comprises the steps of the process as described and claimed in the appended claims and the equivalents thereof.

In the manufacture of viscose, the cellulose comes to the plant in the form of flat sheets resembling cardboard, which are about 16" x 18" in size and about .03" in thickness. These sheets are first steeped in an aqueous solution containing about 18% by weight of sodium hydroxide. The sheets, before soaking, are of the same general size and appearance irrespective of whether the cellulose is made from wood pulp by the sulphite process or from cotton linters treated with a sodium carbonate solution.

The soaking is generally done in sheet metal steeping tanks of various designs. In most instances the tank is provided with a press plate connected to a hydraulic press piston. The sheets are generally stacked vertically in the tank with a perforated metal sheet between every 30 or 40 sheets and the lye solution is then admitted. These per-

forated plates preserve the shape of the soaked cellulose sheets and also assist in letting out the excess lye solution when the sheets are later pressed with the hydraulic piston.

This soaking process requires about one hour after which the hydraulic piston presses out the excess lye to such a degree that the final material contains about 2 to 3 pounds of lye solution for each pound of the original dry cellulose.

In the former processes the pressed cellulose sheets were charged into shredders of various designs, which shredded the cellulose into a white fluffy mass. This shredding process required about two hours, and it was necessary to watch this process very closely, as any temperature rise above 25 degrees centigrade was detrimental to the final product; therefore, these shredders had to be jacketed and cooled by circulating water or brine.

In the shredding operation the size of the batch was considerably limited owing to the temperature rise in the material due to the friction of the shredding blades and the necessity of bringing the material in rapid contact with the cooled walls of the shredder.

As any increment in the size of the shredder greatly increases the capacity in proportion to the increased area, experience has established a limit for the size of the batch beyond which it is dangerous to go, owing to the longer time required by the mixing action of the shredder blades to bring the material from the center of the batch into contact with the cooled walls of the trough.

After leaving the shredders, the cellulose was placed in aging cans where it was left for about 100 hours at a temperature of 25 degrees centigrade. During this aging process, the cellulose decreased slightly in fluffiness as the material settled.

When sufficiently aged, the cellulose was charged into xanthating drums where a measured of weighed quantity of liquid carbon disulphide was then admitted. In these drums the material was tumbled about at a temperature of about 25 degrees centigrade in contact with the carbon disulphide, both

in the liquid and vapor phase. Very shortly after the carbon disulphide had been added the originally pure white material took on an intensely yellow color, caused by the 5 action of the carbon disulphide with the shredded soda cellulose. As the reaction progressed, the fluffy material settled more and more, and the mass became denser and in the form of lumpy dough, due to the tumbling 10 action of the drums.

The xanthate, thus formed, has a "crust" or denser skin on the outside of the lumps which prevented the carbon disulphide from properly acting on the center and which 15 crust, being difficult to dissolve in the later stages, left minute particles in the finished product which were hard to filter, and consequently owing to this and other unknown conditions all batches were not uniform and 20 many batches were lost entirely.

The excess carbon disulphide was then removed after about two to three hours by applying vacuum to the xanthating drums. This step in the process had to be done very 25 carefully because the vapor of carbon disulphide is very explosive when mixed with air.

After removal of the excess carbon disulphide the finished xanthate was immediately 30 dissolved in a dilute lye solution. This dissolving process required considerable additional time and care as well as special machinery to thoroughly dissolve it, and it was rapidly circulated in the lye solution as 35 well as sheared in order to facilitate rapid dissolution and insure a lump free viscose. From this process the finished material went to the filters, further aging, and spinning or casting machines which converted it into the 40 finished product.

The many advantages and values of my invention over the above process will be apparent when compared with the following description of my new process.

45 In the drawing the single figure is a flow diagram showing the progress of the various materials through the several steps of the process according to my invention, the equipment used in this process being shown diagrammatically.

50 Referring now to the drawing, I take the cellulose sheets, soak them in sodium hydroxide for the usual time in the usual steeping tank 1 and press out the excess liquor by the usual press 2.

In actual operation the press is generally constructed as part of the tank, but for the sake of clearness I have shown the press as a separate unit as it forms a separate step in 55 the process.

The pressed sheets are then charged into aging cans 3, where they are left for about 100 hours at a temperature of 25 deg. centigrade.

60 After the cellulose sheets have been prop-

erly aged, they are charged into a mixing and kneading machine of the type shown in U. S. Patent No. 1,632,975 issued June 21, 1927, to Fritz Kempfer. This machine comprises a trough 4, having a plurality of arcuate bottoms 5—5, and a power driven kneading blade 6, coaxial with each compartment located above the arcuate bottoms 5—5, and a rotary impeller 7, which may be raised during the first stages of the kneading process and lowered, to agitate and thoroughly mix the material during the later stages. The mixing and kneading machine is generally driven by a two speed motor, not shown.

As soon as the material has been charged into this kneading machine, with the blades running preferably at slow speed, a cover 8, is tightened down and a vacuum of about 20 to 25 inches is created in the machine by means of a vacuum pump 9. The vacuum pump is then shut off and carbon disulphide is gradually admitted while the machine is under vacuum to lessen the dangers of explosion. The kneading blades are reversed every 20 minutes for a period of two minutes throughout this entire mixing process. The temperature of the material is regulated in proper limits by the admission of a temperature controlling fluid in the jacket 10, of the mixer trough 4.

The action of the kneading blades on the blocks of soda cellulose will first convert them into a loose mass which practically fills the total available space in the equipment. However, as the xanthating process proceeds, due to the gradual admission of the carbon disulphide, the mix becomes denser until finally a smooth plastic xanthate dough of uniform density is formed which is about the consistency of a stiff bread dough. This 95 step of the process requires about two hours.

The excess carbon disulphide is now removed by the application of vacuum to the apparatus and dilute lye is gradually admitted to the xanthate dough which is under proper temperature control. As the dough begins to thin down and form a semi-liquid, the speed of the kneading blades is increased to approximately twice the speed used in the 100 first stage of this step.

The impeller blade 7, is then lowered into the liquid and with this combined stirring action of the impeller blade 7, and kneading action of the mixing blades 6, the xanthate is converted into a liquid, smooth, lump free 105 viscose which is now ready for the filtering, further aging, and spinning or casting process.

The addition of the carbon disulphide and dilute lye to the mass is so gradual that it is 110 thoroughly incorporated by the mixing and stirring blades and consequently the minute lumps found in the viscose made by other processes are entirely eliminated.

115 By the above process I have been enabled 120

to produce a viscose in a much shorter time than has been done heretofore.

I have eliminated several of the steps in the process, particularly the shredding process with its inherent dangers of overheating and limitation of batch size. I have also eliminated the xanthating drum, the explosive hazards attendant upon their operation and the formation of lumps and their crusts which tend to make batches of irregular quality. The dissolving process used heretofore has also been eliminated, and with it the inherent difficulty of eliminating the minute lumps which are difficult to filter, and as some of the lumps find their way through the filters the spun thread is greatly weakened.

I have also saved much time by the elimination of a great deal of the handling required, to transfer the material from one piece of equipment to another, removed many of the dangers of spoiling the batch by overheating, and have enabled the manufacturer to handle larger batches, and at the same time I have produced a viscose in which all batches are uniform, which is easily filterable, and from which a cleaner and stronger rayon thread and a clearer more uniform sheet of cellophane may be manufactured.

Having thus described my invention, what I claim and desire to secure by Letters Patent is:

1. The process of making viscose which consists in soaking cellulose sheets in sodium hydroxide, pressing out the excess sodium hydroxide, aging the soaked and pressed cellulose sheets, kneading the aged cellulose in a vacuum while gradually adding carbon disulphide until the cellulose forms a stiff xanthate dough, removing the excess carbon disulphide by vacuum, gradually adding to the xanthate dough a dilute caustic soda solution while kneading until the xanthate becomes semi-liquid and then stirring and kneading at increased speed until all the caustic soda solution has been added.

2. The process of making viscose which consists in kneading soaked, pressed and aged cellulose sheets while gradually adding carbon disulphide until the cellulose forms a stiff xanthate dough, removing the excess carbon disulphide by vacuum, gradually adding to the xanthate dough a dilute caustic soda solution while kneading until the xanthate becomes semi-liquid and then stirring and kneading until all the caustic soda solution has been added.

3. The process of making viscose which consists in kneading and stirring in a vacuum, soaked, pressed and aged cellulose sheets while gradually adding carbon disulphide until the cellulose forms a stiff xanthate dough, removing the excess carbon disulphide by vacuum, gradually adding a dilute caustic soda solution to the xanthate dough while

kneading and stirring until the xanthate dough becomes semi-liquid, and then increasing the kneading and stirring speed until all the dilute caustic soda solution has been added.

4. The process of making viscose which consists of kneading and stirring soaked, pressed and aged cellulose sheets while gradually adding carbon disulphide until a stiff xanthate dough is formed, removing the excess carbon disulphide by vacuum, and gradually adding a dilute caustic soda solution, while stirring and kneading, until a smooth, lump free, uniform viscose is formed.

In testimony whereof I affix my signature. 80  
RICHARD THURM.

70

85

90

95

100

105

110

115

120

125

130